

## UNITED STATES PATENT OFFICE

2,329,324

## LUBRICANT COMPOSITION

Henry G. Berger, Woodbury, and Francis M. Seger, Pitman, N. J., assignors to Socony-Vacuum Oil Company, Incorporated, New York, N. Y., a corporation of New York

No Drawing. Application May 22, 1941,  
Serial No. 394,616

3 Claims. (Cl. 252—48)

This invention has to do with lubricant compositions and is more particularly concerned with lubricants adapted for use under extreme pressure conditions such as are encountered between relatively moving engaged surfaces in various types of modern machinery, such as the hypoid gears in motor vehicles.

The present invention contemplates a lubricant comprised of a suitable carrying medium such as mineral oil which may or may not have inherent lubricant properties and a dissolved or suspended ingredient which will impart to the composition the property of lubricating metal surfaces engaged under extreme pressures. The carrying medium is preferably a material either in the nature of a liquid or a grease, which preferably has lubricant properties. Viscous mineral oils are representative of such a preferred carrying medium. It is to be understood, however, that the invention is not limited to this particular type of carrying medium but contemplates any medium of suitable volatility in which the extreme pressure ingredient or "E. P. base" can be dissolved, dispersed, or emulsified. Other typical carrying agents contemplated herein are relatively non-viscous petroleum hydrocarbons such as kerosene, and fatty vegetable or animal oils, alcohols, esters, ethers, etc.

Among the various bases or ingredients which have heretofore been proposed for the compounding of extreme pressure lubricants are organic compounds containing chlorine and sulfur in chemical combination. The novel compounds or reaction products contemplated herein may be considered as falling roughly into that general class of compounds, but they are characterized by the fact that the active constituents (chlorine and sulfur) predominate over the organic (carbon) constituent. The materials contemplated for use in compounding the novel lubricant compositions described herein are obtained by reacting perchloromethylmercaptan ( $\text{Cl}_3\text{C.SCl}$ ) with elementary sulfur. This reaction gives rise to a number of reaction products, believed to be a complex mixture of trichloromethyl polysulfides with unreacted  $\text{Cl}_3\text{C.SCl}$ , by-product  $\text{S}_2\text{Cl}_2$ , and various decomposition products of  $\text{Cl}_3\text{C.SCl}$  and the polysulfides, such as  $\text{CCl}_4$ ,  $\text{CSCl}_2$ ,  $\text{S}$ ,  $\text{CS}_2$  and  $\text{SCl}_2$ . For this reason the material contemplated herein as an addition agent for lubricant compositions must be characterized as a reaction product rather than a definite chemical compound, but neglecting the concurrent reactions which give rise to decom-

position products it is believed that the reaction can be roughly represented as follows:



5 The general procedure for obtaining the reaction products contemplated herein involves the reaction of from 2 to 6 parts of perchloromethylmercaptan with 1 part of elementary sulfur at a reaction temperature between 140° and 170° C. 10 This is calculated to give from 6 to 2, respectively, as the value of  $x$  in the formula  $(\text{Cl}_3\text{C})_2\text{S}_x$ , which represents the average composition of the polysulfides in the mixture.

15 Since some of the constituents in the reaction product (such as the  $\text{S}_2\text{Cl}_2$  by-product, unreacted  $\text{Cl}_3\text{C.SCl}$  and decomposition products of  $\text{Cl}_3\text{C.SCl}$ ) are of relatively high volatility, it is desirable to top the crude reaction product for most satisfactory results. Thus, the crude reaction mass 20 may, if desired, be topped at about 100° C. pot temperature at 2 mm. Hg. to remove the more volatile constituents, including  $\text{S}_2\text{Cl}_2$  and unreacted  $\text{Cl}_3\text{C.SCl}$ .

25 As aforesaid, the principal object of this invention is the development of extreme pressure lubricant compositions and with that in mind our invention contemplates the use of any carrying agent wherein a minor proportion of reaction product herein described can be dissolved, dispersed or emulsified. We have discovered, however, that these reaction products, when added to viscous mineral oils, are effective to impart desirable properties other than increased load-carrying capacity. For example, reaction products of the class described, or fractions thereof, may be used in viscous mineral oil fractions in amounts less than those normally desired for extreme pressure properties, to inhibit or retard the deleterious effects of oxidation on such oils as evidenced by reduction in acid formation in highly refined transformer oils and reduction in corrosion of alloy bearings in solvent-refined motor oils.

40 Perchloromethylmercaptan, as indicated by the formula above, is a chlorinated substituted sulfur chloride and can be prepared by the chlorination of carbon disulfide according to the method of Helfrich and Reid (Jour. Amer. Chem. Soc. 43, 591 (1921)). For example, carbon disulfide containing about .4 per cent by weight of iodine was chlorinated in the absence of direct sunlight at a temperature maintained below 25° C. until the volume of the reaction mixture had doubled. The crude product, which has been topped to remove carbon tetrachloride and sulfur dichlo-

ride, is predominantly perchloromethylmercaptan with some sulfur monochloride. This crude product can be used in the preparation of the reaction products contemplated herein, or it may be purified by fractionation.

As aforesaid, the addition agents contemplated herein are preferably obtained by reacting from two to six parts of perchloromethylmercaptan with one part of sulfur, and the reaction is best carried out at elevated temperatures of from about 145° to about 170° C. with the heated reaction mixture under a reflux condenser. The product may be fractionated and purified as herein-after indicated or, if desired, after initial topping, it may be treated (as by water-washing) to destroy traces of sulfur chloride and further treated (as by dilution with petroleum ether) to precipitate elementary sulfur, and then blended with the oil or other carrying medium in the proportions desired for the particular result to be accomplished.

Further details in procedures for preparing reaction products of the type contemplated herein and indications as to their effectiveness as addition agents for lubricant compositions may be obtained from the following examples:

#### Example I

A reaction mixture consisting of 32 grams (1.0 atom) of sulfur and 203 grams (1.1 moles) of crude  $\text{Cl}_3\text{C}\cdot\text{SCl}$  (steam-distilled but not fractionated) was heated under reflux to an initial pot temperature of 110° C.; and after a small amount of low-boiling material was taken off, the temperature rose to 147° C. and was held at 146-163° C. for a total of 9 hours. The take-off condensed during these operations was only 8 grams. On steam-treatment, only 8 grams of steam distillate was obtained. A 5 per cent blend in lubricating oil of the non-volatile product of this reaction tested 570+ pounds on the S. A. E. test machine (described in S. A. E. Journal 39, 23-4 (1936)), and in the Almen test (Proc. A. P. I., 1932, pages 118-130) this blend tested 30,000+ pounds.

The foregoing reaction product, which analyzed 50.5 per cent chlorine and 38.3 per cent sulfur, was distilled under vacuum (1 mm. Hg.), and 60 per cent came over at 107-160° C. The other 40 per cent was left undistilled. The distillate analyzed 57.1 per cent Cl and 35.3 per cent S. Calculated values for bis trichloromethyl tetrasulfide ( $(\text{Cl}_3\text{C})_2\text{S}_4$ ) are 58.4 per cent chlorine and 35.1 per cent sulfur.

#### Example II

A reaction mixture consisting of 48 grams (1.5 atoms) of sulfur and 187 grams (1.0 mole) of perchloromethylmercaptan (B. P. 80-81° C./90 mm. Hg.) was heated under reflux for a total of about 11 hours at a temperature of from 145° to 168½° C. Eighty-eight grams of distillate were then taken off below 92° C. at 7 mm. pressure and discarded. The residual material was fractionally distilled to give the following two fractions:

(1) 51 grams boiling at 40-130° C. at 0.4 mm. pressure and analyzing 63.9 per cent Cl and 29.9 per cent S. A 3 per cent blend of the fraction in lubricating oil gave an S. A. E. test value of 385 pounds and an Almen test value of 29,000 pounds.

(2) 34 grams boiling at 100-175° C. at 0.4 mm. pressure and analyzing 60.3 per cent chlorine and 35.6 per cent sulfur. A 3 per cent blend of

this fraction in lubricating oil gave an S. A. E. test value of 365 pounds and an Almen test value of 28,000 pounds.

#### Example III

5 A reaction mixture consisting of 48 grams (1.5 atoms) of sulfur and 186 grams of perchloromethylmercaptan was heated under reflux for a total of 13½ hours at a temperature of from 139½ to 166½° C. In this run, as in the preceding runs, the temperature of the mixture at reflux showed a characteristic sharp rise followed by a gradual decline. Vapor loss was again negligible. Seventy-six grams of distillate taken below 135° C. pot temperature at 90 mm. pressure was discarded. The residual material was then stirred with water, taken up in petroleum ether, filtered and topped. This product was fractionally distilled to give the following two fractions:

(1) 53 grams of distillate boiling at 50-120° C. at 25 mm. pressure, which in 3 per cent blend in lubricating oil gave an S. A. E. test value of 350 pounds and an Almen test value of 30,000 pounds.

(2) 43 grams of distillate boiling at 120-140° C. at 0.2 mm. pressure. This fraction in a 3 per cent blend in lubricating oil gave an S. A. E. test value of 540 pounds and an Almen test value of 30,000 pounds.

30 From the foregoing it will be seen that the crude product obtained by the reaction of perchloromethylmercaptan and sulfur, together with the various products obtained by fractionating and refining such crude product, are all effective 35 extreme pressure agents, and it is to be understood that where the term reaction product is used herein, such term is intended to include the various fractions typified by those described in 40 the examples either alone or in admixture with the other products of reaction.

As aforesaid, the reaction products contemplated herein have also been demonstrated to be effective to inhibit the deleterious effects of 45 oxidation on refined viscous petroleum oils of the type used as lubricants and dielectrics. For example, fraction 2 from Example IV was blended in an amount of 0.25 per cent in a solvent-refined 50 motor oil, and the blend and blank oil were subjected to a bubble test to demonstrate corrosiveness 55 toward cadmium-silver bearing metals. The blank showed a weight loss of 32 mg. in a 6-gram bearing section, while the blend showed a loss of only 1 mg. on the same-sized section of the same bearing. The fraction 1 from Example IV showed 60 a 4 mg. loss in bearing weight with a 0.25 per cent blend as against a 48 mg. loss for the blank oil. Blends of a highly refined transformer oil containing 0.1 per cent of these same fractions were 65 subjected to a modified German tar test, and the following neutralization numbers (N. N.) were obtained:

|    | Product added               | N. N. |
|----|-----------------------------|-------|
| 65 | None                        | 25.00 |
|    | 0.1% fraction 1, Example IV | 1.2   |
|    | 0.1% fraction 2, Example IV | 0.04  |

70 The amount of the reaction product used will vary depending upon the carrying agent and the purpose for which it is added. When used in viscous mineral oil fractions where an extreme pressure lubricant composition is desired, the amount may be varied from ½ to 10 per cent;

and when added for the sole purpose of inhibiting oxidation the amount will vary from .01 per cent to .50 per cent. In general, therefore, as regards mineral oil compositions, our invention contemplates proportions of the reaction product ranging from 0.01 to 10.0 per cent.

It is to be understood that while we have herein described various procedures for obtaining and purifying the reaction products contemplated herein, the invention is not limited to the details of such procedures but includes within its scope such changes and modifications as fairly come within the spirit of the appended claims.

We claim:

1. A lubricant composition comprising a hydro-carbon lubricating oil and in admixture therewith a minor proportion of the product obtained by refluxing from two to six parts of perchloromethylmercaptan with one part of sulfur at a temperature of from 145° to 170° C.

2. A lubricant composition comprising a hydro-carbon lubricating oil and in admixture therewith a minor proportion of the product obtained by refluxing from two to six parts of perchloromethylmercaptan with one part of sulfur at a temperature of from 145° to 170° C., and then removing sulfur chloride and unreacted sulfur from the reaction product.

3. A lubricant composition comprising a hydro-carbon lubricating oil and in admixture therewith a minor proportion of from 0.01 per cent to 10.0 per cent of the product obtained by refluxing from two to six parts of perchloromethylmercaptan with one part of elementary sulfur at a temperature of from 145° C. to 170° C., and then removing sulfur chloride and unreacted sulfur from the reaction product.

HENRY G. BERGER.  
FRANCIS M. SEGER.